

PATENTED

SEP 29 1868

82507

T. E. Wood. *Elastic Roofing.*



Witnesses.

J. C. Ashketto  
J. A. Fraser

Inventor:

T. E. Wood  
byer Murray  
attorneys

# UNITED STATES PATENT OFFICE.

THOMAS E. WOOD, OF KNOXVILLE, PENNSYLVANIA.

## IMPROVEMENT IN ELASTIC ROOFING COMPOSITIONS.

Specification forming part of Letters Patent No. 82,507, dated September 29, 1868.

*To all whom it may concern:*

Be it known that I, THOMAS E. WOOD, of Knoxville, in the county of Tioga and State of Pennsylvania, have invented a new and useful Improvement in Elastic Roofing; and I do hereby declare that the following is a full, clear, and exact description thereof, which will enable others skilled in the art to make and use the same, reference being had to the accompanying drawings, forming part of this specification.

The nature of my invention relates to improvements in roofing; and consists in the construction of roofs of the compound which will be hereinafter described, when the same is applied in the manner which will be more fully shown on reference to the accompanying drawings, wherein is shown a sectional view of a roof composed of the several constituent parts or chemical elements constituting my invention, and applied in the manner which I have found best adapted to the same.

A represents the portion of a building to be covered. B represents the strips of felting, as commonly used for roofing purposes, laid on in the following manner: Commencing at the eaves, the first sheet is folded under about one-third of its breadth, the second laid on with its lower edge even with the eave, and projecting above the upper edge of the first about one-third its breadth, and the third

sheet commencing with its lower edge laid one-third its breadth above the eaves, so that all parts of the roof are covered with three thicknesses of felt, the whole being laid in hot cement and fastened to the roof by strips of wood or tin laid on at proper distances apart, and secured with nails. I then cover the whole with the elastic compound, prepared as follows: One part asphaltum to six parts gas-tar, to be heated boiling hot; then add five parts clean sand, one part boiled plaster, and one part common paint, to be mixed to the consistency of mortar, and while hot spread on with a trowel from one fourth to one-half inch in thickness, which constitutes, as I have found in practice, a very durable elastic roofing material, which is not liable to crack after it has become hard, or to be affected by the heat of the sun in warm weather.

Having thus fully described my invention, what I claim, and desire to secure by Letters Patent, is—

The elastic roofing composition made of the ingredients and in the proportions herein specified, compounded and applied in the manner set forth.

THOMAS E. WOOD.

Witnesses:

E. P. MASTERSON,  
NOAH EVERITT.